



US006593844B1

(12) **United States Patent**  
Iwao et al.

(10) **Patent No.:** US 6,593,844 B1  
(45) **Date of Patent:** Jul. 15, 2003

(54) **PTC CHIP THERMISTOR**

(75) Inventors: **Toshiyuki Iwao; Koichi Morimoto,**  
both of Osaka; **Kiyoshi Ikeuchi,**  
**Hyogo; Junji Kojima; Takashi Ikeda,**  
both of Osaka, all of (JP)

(73) Assignee: **Matsushita Electric Industrial Co., Ltd.,** Osaka (JP)

(\*) Notice: Subject to any disclaimer, the term of this patent is extended or adjusted under 35 U.S.C. 154(b) by 0 days.

(21) Appl. No.: **09/868,028**

(22) PCT Filed: **Oct. 15, 1999**

(86) PCT No.: **PCT/JP99/05706**

§ 371 (c)(1),  
(2), (4) Date: **Jun. 13, 2001**

(87) PCT Pub. No.: **WO00/24010**

PCT Pub. Date: **Apr. 27, 2000**

(30) **Foreign Application Priority Data**

Oct. 16, 1998 (JP) ..... 10-294946  
Jun. 1, 1999 (JP) ..... 11-153292

(51) **Int. Cl. 7** ..... **H01C 7/10**

(52) **U.S. Cl.** ..... **338/22 R; 338/328; 338/332**

(58) **Field of Search** ..... **338/22 R, 225 D, 338/328, 332**

(56) **References Cited**

## U.S. PATENT DOCUMENTS

4,290,041 A \* 9/1981 Utsumi et al. ..... 338/21  
5,075,665 A \* 12/1991 Taira et al. ..... 338/21  
5,245,309 A \* 9/1993 Kawase et al. ..... 338/22 R  
6,008,717 A \* 12/1999 Kawase et al. ..... 338/22 R  
6,020,808 A \* 2/2000 Hogge ..... 338/22 R  
6,023,403 A 2/2000 McGuire et al.  
6,078,250 A \* 6/2000 Ueda et al. ..... 338/313  
6,157,289 A \* 12/2000 Kojima et al. ..... 338/22 R  
6,172,591 B1 \* 1/2001 Barrett ..... 338/22 R  
6,184,769 B1 \* 2/2001 Nakamura et al. ..... 338/21  
6,188,308 B1 \* 2/2001 Kojima et al. ..... 338/22 R  
6,236,302 B1 \* 5/2001 Barrett et al. ..... 338/22 R  
6,242,997 B1 6/2001 Barrett et al.

## FOREIGN PATENT DOCUMENTS

|    |          |         |
|----|----------|---------|
| JP | 4-346409 | 12/1992 |
| JP | 6-061014 | 3/1994  |
| JP | 6-44101  | 6/1994  |
| JP | 6-208903 | 7/1994  |
| JP | 9-69416  | 3/1997  |
| JP | 9-503097 | 3/1997  |
| JP | 10-12404 | 1/1998  |
| WO | 98/12715 | 3/1998  |

## OTHER PUBLICATIONS

International Search Report corresponding to application No. PCT/JP99/05706 dated Jan. 25, 2000.

English translation of PCT/ISA/210, Sep. 14, 2000.

International Search Report for PCT/JP00/01228 dated Jun. 6, 2000.

English translation of PCT/ISA/210 Jun. 6, 2000.

\* cited by examiner

Primary Examiner—Karl D. Easthom

(74) Attorney, Agent, or Firm—RatnerPrestia

(57) **ABSTRACT**

A chip PTC thermistor comprising a conductive polymer having PTC properties, a first outer electrode, a second outer electrode, one or more inner electrodes sandwiched between the conductive polymer, a first electrode electrically directly coupled with the first outer electrode, and a second electrode. The odd-numbered inner electrode among the one-or-more inner electrodes is directly coupled with the second electrode, while the even-numbered inner electrode, with the first electrode. When total number of the inner electrodes is an odd number the second outer electrode makes direct electrical contact with the first electrode, when it is an even number the second outer electrode makes direct electrical contact with the second electrode. Defining a distance from the odd-numbered inner electrode to the first electrode, or from the even-numbered inner electrode to the second electrode, as “a”, while a distance between the adjacent inner electrodes, or a distance between the inner electrode placed the most adjacent to the first outer electrode, or the second outer electrode, and the first outer electrode, or the second outer electrode, as “t”; the PTC thermistors are constituted so that a ratio  $a/t$  is within 3–6. The chip PTC thermistors in accordance with the present invention effectively prevent an overcurrent in large current circuits.

14 Claims, 19 Drawing Sheets



FIG. 1



FIG. 2



FIG. 3



FIG. 4



FIG. 5



FIG. 6



FIG. 7



FIG. 8



FIG. 9

(a)



(b)



(c)



FIG. 10

(a)



(b)



(c)



FIG. 11



FIG. 12



FIG. 13



FIG. 14



FIG. 15

(a)



(b)



(c)



FIG. 16

(a)



(b)



(c)



FIG. 17



FIG. 18



FIG. 19



FIG. 20



## PTC CHIP THERMISTOR

THIS APPLICATION IS A U.S. NATIONAL PHASE APPLICATION OF PCT INTERNATIONAL APPLICATION PCT/JP99/05706.

## FIELD OF THE INVENTION

The present invention relates to a chip positive temperature coefficient (hereinafter, PTC) thermistor comprising conductive polymers having PTC properties. The present invention particularly relates to a laminated chip PTC thermistor.

## BACKGROUND OF THE INVENTION

PTC thermistors have been used as an overcurrent protection element. When an electric circuit gets overloaded, conductive polymers of a PTC thermistor, which have PTC properties, emit heat and thermally expand to become high resistance, thereby reducing the current in the circuit to a safe small current level.

The following is a description of a conventional laminated chip PTC thermistor (hereinafter, PTC thermistor).

The Japanese Patent Application Laid Open Publication No. H9-69416 discloses a structure of the conventional chip PTC thermistors. A conductive polymer sheet and an internal electrode of metal foil are alternately laminated so that number of the conductive polymer sheets is more than two, for providing a PTC thermistor element. Terminals coupled respectively with the opposing internal electrodes are provided on opposite side faces to complete a finished chip PTC thermistor.

FIG. 20 is a cross section of a conventional chip PTC thermistor. Referring to FIG. 20, a conductive polymer 1 is formed of polyethylene or the like high polymer sheet material mixed with carbon black or the like conductive particles and cross-linked. Internal electrode 2a, 2b, 2c, 2d made of a conductive material and a conductive polymer sheet 1 are laminated to form a PTC thermistor element 3. Provided on the side faces of the thermistor element 3 are terminals 4a and 4b, which are coupled respectively with the internal electrodes 2a, 2c and 2b, 2d.

However, the above-described structure of conventional PTC thermistors exhibits following problems when they are intended to be made smaller in size, or capable of larger current.

In order to make a PTC thermistor to be compact and capable of handling a large current, the DC resistance of the PTC thermistor needs to be lowered. For reducing the specific resistance of the conductive polymer 1, it is effective to increase amount of the conductive particles contained in the conductive polymer. However, the increased conductive particles also effects a deterioration in the rising rate of the resistance, which being a key PTC characteristic, rendering it difficult to cut off the electric current when an abnormality happens.

The resistance can be lowered also by reducing the thickness of conductive polymer 1 placed among the internal electrodes 2a, 2b, 2c, 2d. However, this measure also leads to a deterioration in the rising rate of the resistance, like in the earlier example, and to a lowered withstand voltage.

Furthermore, the resistance can be lowered also by increasing the opposing area of the internal electrodes 2a, 2b, 2c, 2d. The opposing area can be increased by increasing the number of laminated layers. However, the increased layers result in a greater thickness with a laminated body,

which readily leads to a lower reliability in the connection between the internal electrodes 2a, 2b, 2c, 2d and the terminals 4a, 4b, being affected by a mechanical stress caused by expansion of the conductive polymer 1. Thus, 5 there is a limitation in the increasing the number of layers.

Therefore, in order to lower the resistance, the effective opposing area per layer must be increased by making the distance between the internal electrodes 2a, 2b, 2c, 2d and the terminals 4a, 4b shorter. However, the portion of the 10 conductive polymer 1 locating in the vicinity of the terminals 4a, 4b is physically restricted by the internal electrodes 2a, 2b, 2c, 2d, which means that it is not easy for the conductive polymer 1 to expand. As a result, when an overcurrent causes an expansion with the conductive polymer 1, the expansion remains small in the vicinity of the terminals 4a, 4b, leaving the specific resistance in the region to be small as compared with that in other regions. So, the rising rate of the resistance is impaired with a PTC thermistor whose distance between the internal electrodes 2a, 2b, 2c, 2d and the terminals 4a, 4b is short. Thus, the PTC thermistors had a problem that there is a possibility for the 20 rising rate of the resistance to become low, if lowering of the resistance is intended to be realized through introduction of a laminated structure and increase in the effective opposing area.

The present invention addresses the above drawbacks, and aims to provide a chip PTC thermistor that is compact in shape, yet it is usable in the large current applications with a sufficient rising rate in the resistance.

## SUMMARY OF THE INVENTION

A chip PTC thermistor of the present invention comprises:

- a) a conductive polymer having PTC properties;
- b) a first outer electrode in contact with the conductive polymer;
- c) a second outer electrode sandwiching the conductive polymer with the first outer electrode;
- d) one or more inner electrode disposed in between and parallel to the first and second outer electrodes and sandwiched with the conductive polymer;
- e) a first electrode electrically directly coupled with the first outer electrode; and
- f) a second electrode disposed electrically independently from the first electrode.

Where; when counting from one inner electrode, which is the closest to the first outer electrode, an inner electrode in the "n"th position is called as the "n"th inner electrode. If "n" is an odd-number, the inner electrodes are directly 50 coupled with the second electrode; whereas, if "n" is an even-number, the inner electrodes are directly coupled with the first electrode. When the total number of the inner electrodes is an odd number, the second outer electrode is electrically directly coupled with the first electrode; whereas, if the total number of the inner electrodes is an even number, the second outer electrode is electrically directly coupled with the second electrode.

In the above PTC thermistor, distance from the odd-numbered inner electrode to the first electrode, or that from 60 the even-numbered inner electrode to the second electrode, is defined as "a",

while distance among the adjacent inner electrodes, or distance from an inner electrode, locating next to the first outer electrode or the second outer electrode, to the first outer electrode, or the second outer electrode, is defined as 65 "t",

"a" and "t" satisfy a relation of  $a/t=3-6$ .

In accordance with a structure that meets the above-described requirement, resistance of a PCT thermistor can be maintained low, and, at the same time, the rising rate of the resistance can be made sufficiently high. Thus the PCT thermistors of the present invention can be used for large current applications despite their compact size, and provide a sufficient capability for preventing an overcurrent. The terminology, "the rising rate of the resistance", used here with a PTC thermistor is defined as a ratio of resistance at an overcurrent divided by resistance at a normal current. The PTC thermistors in accordance with the present invention obtains the above-described functions and capabilities by controlling the parameters to be  $a/t=3-6$ .

#### BRIEF DESCRIPTION OF THE DRAWINGS

FIG. 1(a) is a perspective view of a PTC thermistor in accordance with a first exemplary embodiment of the present invention.

FIG. 1(b) is a sectional view, sectioned at A-A' line of FIG. 1(a).

FIGS. 2(a)-(c) are flow charts showing a method of manufacturing a PTC thermistor in the first embodiment.

FIGS. 3(a)-(e) are flow charts showing a method of manufacturing a PTC thermistor in the first exemplary embodiment.

FIG. 4(a) is a graph showing an example of the resistance-temperature relationship in the first exemplary embodiment.

FIG. 4(b) is a graph showing results of measurement at 125° C. in the first exemplary embodiment.

FIG. 5 is a cross sectional view of a PTC thermistor in the first exemplary embodiment.

FIGS. 6(a), (b) are cross sectional views showing another PTC thermistor samples in accordance with the first exemplary embodiment.

FIG. 7 is a cross sectional view showing still another example in the first exemplary embodiment.

FIG. 8 is a cross sectional view showing a PTC thermistor in accordance with a second exemplary embodiment.

FIGS. 9(a)-(c) are flow charts showing a method of manufacturing a PTC thermistor in the second exemplary embodiment.

FIGS. 10(a)-(c) are flow charts showing a method of manufacturing a PTC thermistor of in the second exemplary embodiment.

FIG. 11 is a cross sectional view showing a PTC thermistor in accordance with the second exemplary embodiment.

FIGS. 12(a), (b) are cross sectional views of PTC thermistors in the second exemplary embodiment.

FIG. 13 is a cross sectional view showing another example of PTC thermistor in accordance with the second exemplary embodiment.

FIG. 14 is a cross sectional view showing a PTC thermistor in accordance with a third exemplary embodiment.

FIGS. 15 (a)-(c) are flow charts showing a method of manufacturing a PTC thermistor in the third exemplary embodiment.

FIGS. 16(a)-(c) are flow charts showing a method of manufacturing a PTC thermistor in the third exemplary embodiment.

FIG. 17 is a cross sectional view showing a PTC thermistor in accordance with the third exemplary embodiment.

FIGS. 18(a), (b) are cross sectional views of PTC thermistors in the third embodiment.

FIG. 19 is a cross sectional view showing another example of PTC thermistor in accordance with the third exemplary embodiment.

FIG. 20 is a cross sectional view of a conventional PTC thermistor.

#### DESCRIPTION OF THE PREFERRED EMBODIMENTS

##### First Exemplary Embodiment

A PTC thermistor in accordance with the first exemplary embodiment of the present invention is described referring to the drawings.

FIG. 1(a) is a perspective view of a PTC thermistor in accordance with the first exemplary embodiment of the present invention and FIG. 1(b) is the cross sectional view, sectioned at the line A-A' of FIG. 1(a).

Referring to FIGS. 1(a) and (b), a conductive polymer 11 is a mixture of a high density polyethylene, which is one of the crystalline polymers, and carbon black, which is a conductive particle. The conductive polymer 11 is provided with the PTC properties. A first outer electrode 12a is provided on a first surface of the conductive polymer 11, and a second outer electrode 12b on a second surface opposite the first surface of the conductive polymer 11. Each of the first and the second outer electrodes is formed of a metal foil, such as copper, nickel or the like. A first electrode 13a comprising a nickel plating layer is provided to cover the entire surface of one of the side faces of the conductive polymer 11 as well as end portions of the first outer electrode 12a and the second outer electrode 12b, electrically coupling them. A second electrode 13b comprising a nickel plating layer is provided to cover the entire surface of the other side face of the conductive polymer 11 as well as end portions of the first and the second surfaces of the conductive polymer 11. A first and a second protective coating 14a and 14b are formed of an epoxy modified acrylic resin, and are provided on the outermost surface of the first and the second surfaces of the conductive polymer 11. A first and a second protective coating 14a and 14b are formed of an epoxy modified acrylic resin, and are provided on the outermost surface of the first and the second surfaces of the conductive polymer 11. An inner electrode 15 is formed of a metal foil, such as copper, nickel and the like, and is provided in the conductive polymer 11, in parallel to the outer electrodes 12a and 12b, and electrically coupled with the side electrode 13b.

A method for manufacturing the above-configured PTC thermistor in accordance with first embodiment is described with reference to the drawings.

FIGS. 2(a)-(c) and FIGS. 3(a)-(e) are process charts showing a method of manufacturing the PTC thermistor in first embodiment.

First, a 0.16 mm thick conductive polymer sheet 21 shown in FIG. 2(a) is manufactured by mixing the following materials in a hot 2-roll mill at approximately 170° C. for about 20 minutes and then the mixture is pulled out of the 2-roll mill in the form of a sheet:

a 42 weight % (wt %) of high density polyethylene, having a crystallinity of 70-90%,

a 57 wt % of furnace carbon black, having an average particle diameter of 58 nm, specific surface area of 38 m<sup>2</sup>/g, and

a 1 wt % of anti-oxidant.

An electrolytic copper foil of approximately 80  $\mu$ m thick is pressed by a metal mold to form a pattern of electrodes 22 as shown in FIG. 2(b). A groove 28 shown in FIG. 2(b) is for providing gaps between the side electrode and the outer electrode, or the inner electrode, so that the respective electrodes are separated from each other for a predetermined

distance, after being divided into independent pieces in a later process stage. A groove 29 is for preventing burrs on the electrolytic copper foil, by reducing an area of the electrolytic copper foil being cut during the dividing process. The groove 29 also prevents a section of the electrolytic copper foil from being exposed to the outside. If there is an exposed section, it might get oxidized, or introduce short circuiting caused by a solder during mounting of a finished thermistor.

The patterned electrodes 22 form the outer electrode 12a, the outer electrode 12b or the inner electrode 15, in a finished PTC thermistor.

As shown in FIG. 2(c), two conductive polymer sheets 21 and three sheets of patterned electrodes 22 are stacked alternately so that the patterned electrodes 22 come to the outermost layers. The laminate is hot pressed by a vacuum hot press for one minute at 175° C., under a vacuum of 20 Torr, and a pressure of 75 kg/cm<sup>2</sup> to form a first integrated sheet 23 shown in FIG. 3(a).

The first integrated sheet 23 is heat treated (at 110° C.~120° C. for one hour), and then irradiated in an electron beam apparatus at approximately 40 Mrad to cross-link the high density polyethylene.

Then, as shown in FIG. 3(b), a narrow and long opening 24 is provided at a predetermined interval by a dicing tool, in such a manner that a space left between the openings corresponds to length in the longer sides of a finished PTC thermistor.

The first sheet 23 provided with the openings 24 is screen-printed at the top and the bottom surfaces with an UV-curable and heat curable epoxy-modified acrylic resin, excluding a region in the vicinity of the opening 24. Then, the sheet is provisionally cured in a UV-curing oven one surface after the other surface, and then it is finally cured in a heat-curing oven with the both surfaces at once for forming a protective coating 25. The protective coating 25 forms a first protective coat 14a and a second protective coat 14b, in a finished PTC thermistor.

Referring to FIG. 3(d), the first sheet 23 is then wholly immersed in a nickel sulfamate bath and plated with a nickel plating layer of approximately 20  $\mu\text{m}$  thick to form side electrodes 26 by coating portions of the sheet 23, which are not coated with the protective coating 25 and inner walls of the openings 24. Plating conditions are a current density of 4 A/dm<sup>2</sup> and a period of about 40 minutes. The sheet 23 as shown in FIG. 3(d) is then diced into individual elements to complete a finished chip PTC thermistor 27 of the present invention, as shown in FIG. 3(e).

Now in the following, reasons why the ratio a/t needs to be regulated to be within a certain range for a PTC thermistor to obtain a sufficiently high rising rate in the resistance is described in accordance with the present invention; where "a" represents a distance between the side electrode 13a and the inner electrode 15, "t" represents a thickness of the conductive polymer 11 disposed between the inner electrode 15 and the outer electrode 12a, or 12b, in FIG. 1.

As already described, if the distance "a" between the inner electrode 15 and the first side electrode 13a is short, the rising rate of the resistance of a PTC thermistor deteriorates. Therefore, the distance "a" needs to be regulated in order not to introduce the deterioration in the rising rate of the resistance. Meanwhile, the PTC thermistors have been made with a laminated structure in order to obtain a low resistance at the normal temperature; therefore, the distance "a" is not allowed to be very long if the effective opposing area between the outer electrode 12a, or the outer electrode 12b, and the inner electrode 15 should be large enough.

In accordance with the manufacturing method described in the present embodiment, following samples were manufactured: Thickness "t" of the conductive polymer 11 between the outer electrode 12a, or the outer electrode 12b, and the inner electrode 15 is fixed to be 0.15 mm; while electrolytic copper foils are patterned into respective patterns, so that the distance "a" between the side electrode 13a and the inner electrode 15 varies from 0.15 mm to 1.2 mm, at an interval of 0.15 mm.

These samples were tested in order to confirm difference in the rising rate of the resistance that might be caused by the difference in the distance "a".

Five samples each, with which the distance "a" varies from 0.15 mm to 1.2 mm at an interval of 0.15 mm, were mounted on a printed circuit board and placed in a temperature chamber. Temperature of the chamber was raised from 25° C. to 150° C. at a speed of 2° C./min., and the resistance was measured at each temperature. FIG. 4(a) shows an example of the resistance/temperature characteristic, with the samples of 0.15 mm and 0.9 mm with respect to "a". FIG. 4(b) shows a relationship between resistance at 125° C. (R125) and the ratio a/t; "a" the distance, "t" the thickness of the conductive polymer. From FIGS. 4(a) and (b), it has been confirmed that the rising rate of the resistance goes high enough when the value a/t is greater than 3, especially when it is greater than 4. It has also been confirmed that the rising rate of the resistance does not substantially change when the value a/t is 6 or greater, and when the value a/t is 6 or greater, the initial (25° C.) resistance rises.

Since the present invention aims to provide a PTC thermistor that is suitable to the large current applications, the high initial resistance is not preferred. Thus a range of the value a/t suitable to the present invention is; not less than 3, not greater than 6; preferably not less than 4, not greater than 6.

Next, another type of chip PTC thermistor samples were manufactured by providing the conductive polymer sheet 21 on both surfaces of the sheet 23 prepared in accordance with the manufacturing method of present embodiment, where the outer electrodes 12a, 12b are located within the conductive polymer 11. A sheet 23 made by the method as described earlier with the present embodiment is sandwiched with conductive polymer sheets 21 and they are hot pressed. Then, sample chip PTC thermistors were manufactured through the same procedure as described earlier with the present embodiment. FIG. 5 shows a cross sectional view of the chip PTC thermistor. Referring to FIG. 5, thickness "t" of the conductive polymer 11 is fixed at 0.15, while the distance "a" is varied from 0.15 mm to 1.2 mm at an interval of 0.15 mm. The electrolytic copper foils are patterned accordingly. Five samples each were tested in the same manner to measure the resistance at 25° C. and 125° C., and the rising rate of the resistance value was calculated. The results confirm that, like in the earlier samples, the rising rate of the resistance becomes high when the value a/t is greater than 3, especially when it is greater than 4. When the value a/t is greater than 6, the rising rate of the resistance does not show a substantial change, and the initial (25° C.) resistance becomes high.

Next, with an aim to improve reliability in the connection between the outer electrodes 12a, 12b and the side electrode 13a, as well as that between the inner electrode 15 and the side electrode 13b, chip PTC thermistor samples are prepared; in which, as shown in FIGS. 6(a), (b), a first sub electrode 16a is provided on a same plane of the first outer electrode 12a, the electrode 16a being independent from the outer electrode 12a and connected with the side electrode

13b. Also a second sub electrode 16b is provided on a same plane of the outer electrode 12b, the sub electrode 16b being independent from the outer electrode 12b and connected with the side electrode 13b. Furthermore, an inner sub electrode 17 is provided on a same plane of the inner electrode 15, the inner sub electrode 17 being independent from the inner electrode 15 and connected with the first side electrode 13a. The terminology, "independent", means that there is no direct electrical connection, but it does not mean to exclude an electrical coupling via the conductive polymer.

10 The samples were manufactured in the following manner:

Thickness "t" of the conductive polymer 11 was fixed to be 0.15 mm; each of the respective distances between the sub electrode 16a and the outer electrode 12a, between the sub electrode 16b and the outer electrode 12b, between the inner sub electrode 17 and the inner electrode 15 to be longer than 0.3 mm; while a distance "a" between the first side electrode 13a and the inner electrode 15 was varied from 0.45 mm to 1.2 mm, at an interval of 0.15 mm. Electrolytic copper foils were patterned accordingly. Five samples each were tested in the same manner to measure the resistance at 25° C. and 150° C., and the rising rate of the resistance was calculated. The results confirm that, like in the earlier samples, the rising rate of the resistance becomes high when the value a/t is greater than 3, especially when it is greater than 4. When the value a/t is greater than 6, the rising rate of the resistance does not show a substantial change, and the initial (25° C.) resistance becomes high.

In the description of present embodiment, the side electrode 13a and the side electrode 13b have been provided respectively as the first electrode electrically connected with the outer electrode 12a and the outer electrode 12b, and as the second electrode electrically connected with the inner electrode, which inner electrode opposing direct to the first outer electrode. However, the locations for the first electrode and the second electrode are not limited to the side faces of the conductive polymer 11. Instead, the first electrode and the second electrode may be provided in the form of a first penetrating through electrode 18a and a second penetrating through electrode 18b, as shown in FIG. 7.

Namely, in FIG. 7, the conductive polymer 11, the outer electrode 12a, the outer electrode 12b, the protective coating 14a, the protective coating 14b and the inner electrode 15 have been structured the same as those in the first preferred embodiment described above. The difference as compared with the first preferred embodiment (FIG. 1) is that there are a first penetrating through electrode 18a electrically connected with the outer electrode 12a and the outer electrode 12b and a second penetrating through electrode 18b electrically connected with the inner electrode 15, which directly opposing to the outer electrode 12a. The above-configured chip PTC thermistor also provides the same effects as provided by the present invention.

In the foregoing descriptions, the side electrode 13a and the side electrode 13b have been formed covering the whole side faces of the conductive polymer 11, and the edge regions of the outer electrode 12a and the outer electrode 12b, or extending to partly cover the first and the second surfaces of the conductive polymer 11. However, the side electrode 13a and the side electrode 13b may be provided instead on part of the side faces of the conductive polymer 11, to obtain the same effects of the present invention.

The outer electrode 12a, the outer electrode 12b and the inner electrode 15 have been made with a metal foil, in the first embodiment. However, these electrodes can be formed instead by sputtering, plasma spraying or plating of a conductive material. Or, they can be provided by first

sputtering, or plasma spraying a conductive material, and then providing a plating layer thereon. Or, they can be formed using a conductive sheet. The conductive sheet can be a sheet containing either one material among the group of powdered metal, metal oxide, conductive nitride or carbide, and carbon. Furthermore, the electrodes can be formed of a conductive sheet consisting of a metal mesh and either one material among the group of powdered metal, metal oxide, conductive nitride or carbide, and carbon. Either one of the above materials provides the same effects.

#### 10 Second Embodiment

A chip PTC thermistor in accordance with a second exemplary embodiment of the present invention is described with reference to the drawings. FIG. 8 is a cross sectional view of the chip PTC thermistor.

15 In FIG. 8, a conductive polymer 31 is a mixture of a high density polyethylene and carbon black or the like, and has PTC properties. A first outer electrode 32a is disposed on the first surface of the conductive polymer 31, while a second outer electrode 32b is on the second surface. These electrodes are formed of a metal foil, such as copper, nickel or the like. A first side electrode 33a comprising a nickel plating layer is provided covering the entire surface of one of the side faces of the conductive polymer 31 as well as end part of the outer electrode 32a and the edge part of the second face of the conductive polymer 31, and is electrically connected with the first outer electrode 32a. A second side electrode 33b comprising a nickel plating layer is provided covering the entire surface of the other side face of the conductive polymer 11 as well as edge part of the first face of the conductive polymer 31 and end part of the second outer electrode 32b, and is electrically connected with the second outer electrode 32b. A first and a second protective coatings 34a and 34b, formed of an epoxy modified acrylic resin, are provided respectively on the outermost surfaces of the first surface and the second surface of the conductive polymer 31. A first and a second inner electrodes 35a, 35b are provided inside the conductive polymer 31, in parallel with the outer electrode 32a and the outer electrode 32b. The inner electrode 35a is electrically connected with the side electrode 33b, while the inner electrode 35b with the side electrode 33a. These inner electrodes are formed of a metal foil, such as copper, nickel or the like.

20 Now in the following, a method for manufacturing the chip PTC thermistor structured in accordance with the present embodiment is described with reference to the drawings.

25 FIGS. 9(a)–(c) and FIGS. 10(a) and (b) are process charts showing a manufacturing method of a chip PTC thermistor in accordance with second preferred embodiment. In the same way as in the first embodiment, a conductive polymer sheet 41 shown in FIG. 9(a) is prepared. An electrolytic copper foil of approximately 80  $\mu\text{m}$  thick is patterned using a metal mold to form a sheet of electrodes 42 as shown in FIG. 9(b). The sheet of electrodes 42 are provided on both surfaces of the conductive polymer sheet 41 as shown in FIG. 9(c), and then they are pressed under heat and pressure to create a first integrated sheet 43 as shown in FIG. 10(a). Then, the first sheet 43 is sandwiched by two conductive polymers 41, and further by two sheets of electrodes 42, so that the electrodes sheet 42 come to the outermost surface as illustrated in FIG. 10(b). The laminate is pressed under heat and pressure to create a second integrated sheet 44 shown in FIG. 10(c). The rest of the procedure for manufacturing the PTC thermistors of embodiment 2 remains the same as in the first embodiment.

30 Samples were manufactured in accordance with the manufacturing method of the present embodiment in the

following manner: thickness "t" of the conductive polymer 31 was fixed to be 0.15 mm; each of the respective distances "a" between the first and the second inner electrodes 35a, 35b and the first and the second side electrodes 33a, 33b was varied from 0.15 mm to 1.2 mm, at an interval of 0.15 mm. The electrolytic copper foils were patterned accordingly.

In order to confirm difference in the rising rate of the resistance caused by the varied distance, the samples were tested as follows.

Five samples each, with which the distance "a" varies from 0.15 mm to 1.2 mm at an interval of 0.15 mm, were mounted on a printed circuit board to be measured with respect to the resistance/temperature characteristic, in the same manner as in the first embodiment. The results confirm that the rising rate of the resistance becomes high when a value a/t is 3 or greater, especially when it is 4 or greater. It is also confirmed that the rising rate of the resistance does not substantially change when the value a/t is 6 or greater, and when the value a/t is 6 or greater, the initial (25° C.) resistance becomes high. Thus it is confirmed that the results coincide with those of the first embodiment.

Next, another type of chip PTC thermistor samples were manufactured by providing the conductive polymer sheet 41 on both surfaces of the sheet 44 and applying heat and pressure thereon. Thus the outer electrodes 32a, 32b locate within the conductive polymer 31. The rest of the procedure for manufacturing the samples remains the same as that for the above second embodiment. FIG. 11 shows a cross sectional view of the chip PTC thermistor samples. Referring to FIG. 11, thickness "t" of the conductive polymer 11 was fixed at 0.15 mm, while the distance "a" was varied from 0.15 mm to 1.2 mm at an interval of 0.15 mm. Electrolytic copper foils were patterned accordingly. Five samples each were tested in the same manner to measure the resistance at 25° C. and 125° C., and the rising rate of the resistance was calculated. The results confirm that, like in the earlier samples, the rising rate of the resistance becomes high when a value a/t is 3 or greater, especially when it is 4 or greater. It is also confirmed that the rising rate of the resistance does not substantially change when the value a/t is 6 or greater, and the initial (25° C.) resistance becomes high.

Next, with an aim to improve reliability in the connection between the outer electrode 32a, the inner electrode 35b and the first side electrode 33a, as well as that between the outer electrode 32b, the inner electrode 35a and the side electrode 33b, following chip PTC thermistor samples were manufactured. Namely, as shown in FIGS. 12(a) and (b), a first sub electrode 36a is provided on a same plane of the outer electrode 32a, sub electrode 36a being independent from the outer electrode 32a and connected with the side electrode 33b. Also a second sub electrode 36b is provided on a same plane of the outer electrode 32b, sub electrode 36b being independent from the outer electrode 32b and connected with the side electrode 33a. Furthermore, a first inner sub electrode 37a is provided on a same plane of the inner electrode 35a, inner sub electrode 37a being independent from the inner electrode 35a and connected with the side electrode 33a. Still further, a second inner sub electrode 37b is provided on a same plane of the inner electrode 35b, inner sub electrode 37b being independent from the inner electrode 35b and connected with the side electrode 33b.

The samples were manufactured in the following manner: thickness "t" of the conductive polymer 31 was fixed to be 0.15 mm; each of the respective distances between the sub electrode 36a and the outer electrode 32a, between the sub electrode 36b and the outer electrode 32b, between the inner

sub electrode 37a and the inner electrode 35a, and between the inner sub electrode 37b and the inner electrode 35b was provided to be longer than 0.3 mm; and the distance "a" between the inner electrode 35a, 35b and the side electrode 33a, or 33b, was varied from 0.45 mm to 1.2 mm, at an interval of 0.15 mm. Electrolytic copper foils were patterned accordingly. Five samples each were tested in the same manner to have the resistance at 25° C. and 150° C. measured, and the rising rate of the resistance was calculated. The results confirm that, like in the earlier samples, the rising rate of the resistance becomes high when the value a/t is 3 or greater, especially when it is 4 or greater. It is also confirmed that the rising rate of the resistance does not substantially change when the value a/t is 6 or greater, and the initial (25° C.) resistance becomes high.

In the present embodiment, a side electrode 33a and a side electrode 33b have been provided respectively as the first electrode and the second electrode. However, the locations for the first electrode and the second electrode are not limited to the side faces of the conductive polymer 31. Instead, the first electrode and the second electrode can be provided in the form of a first penetrating through electrode 38a and a second penetrating through electrode 38b, as shown in FIG. 13.

Namely, referring to FIG. 13, the conductive polymer 31, the outer electrode 32a, the outer electrode 32b, the protective coating 34a, the protective coating 34b, the inner electrode 35a and the inner electrode 35b have been structured the same as in the earlier examples. The difference is that there are a first penetrating through electrode 38a electrically connected with the outer electrode 32a and a second penetrating through electrode 38b electrically connected with the outer electrode 32b. The above-configured chip PTC thermistors also have the same effects that is provided by the present invention.

The outer electrodes, the side electrodes, the inner electrodes can be provided in the same shape and the same material as in the first embodiment.

#### Third Embodiment

A chip PTC thermistor in accordance with a third exemplary embodiment of the present invention is described referring to the drawings. FIG. 14 is a cross sectional view of the chip PTC thermistor.

In FIG. 14, a conductive polymer 51 is made of a mixture of a high density polyethylene and carbon black or the like, and has a PTC property. A first outer electrode 52a is disposed on a first surface of the conductive polymer 51, while a second outer electrode 52b is on a second surface. These electrodes are formed of a metal foil, such as copper, nickel or the like. A first side electrode 53a comprising a nickel plating layer is provided covering the entire surface of one of the side faces of the conductive polymer 51 as well as end part of the outer electrode 52a and the outer electrode 52b, and is electrically connected with the outer electrode 52a and the outer electrode 52b. A second side electrode 53b comprising a nickel plating layer is provided covering the entire surface of the other side face of the conductive polymer 51 as well as end part of the first surface and the second surface of the conductive polymer 51. A first and a second protective coatings 54a and 54b, formed of an epoxy modified acrylic resin, are provided on the outermost surface of the first surface and the second surface of the conductive polymer 51. A first, a second and a third inner electrodes 55a, 55b, 55c are provided within the conductive polymer 51, in parallel with the outer electrodes 52a, 52b. The inner electrodes 55a, 55c are electrically connected with the side electrode 53b, while the inner electrode 55b is electrically

connected with the side electrode **53a**. These inner electrodes are formed of a metal foil, such as copper, nickel or the like.

Now in the following, a method of manufacturing the above-configured chip PTC thermistors is described with reference to the drawings.

FIGS. 15(a)–(c) and FIGS. 16(a) and (b) are process charts showing manufacturing method of the chip PTC thermistors in accordance with third exemplary embodiment of the present invention. A conductive polymer sheet **61** shown in FIG. 15(a) is prepared in the same way as in the first embodiment. An electrolytic copper foil of approximately 80  $\mu\text{m}$  thick is patterned using a metal mold to provide a sheet of electrodes **62** as shown in FIG. 15(b). The conductive polymer **61** forms the conductive polymer **51** when a finished PTC thermistor is completed; likewise, the electrodes **62** forms the first outer electrode **52a**, the second outer electrode **52b** and the first through the third inner electrodes **55a**–**55c**. Then, as shown in FIG. 15(c), two sheets of the conductive polymer **61** and three sheets of the electrodes **62** are laminated one on the other, so that the electrodes **62** come to the outermost. The laminate is pressed under heat and pressure to prepare an integrated sheet **63** shown in FIG. 16(a). The sheet **63** is sandwiched by two sheets of the conductive polymer **61**, and by two sheets of electrodes **62** so that the electrodes **62** come to the outermost. The laminate is pressed under heat and pressure to prepare an integrated sheet **64** shown in FIG. 16(c). Then, it undergoes the same manufacturing procedure as in the first embodiment, and chip PTC thermistor samples of third embodiment are manufactured.

Now in the following, reasons why the ratio  $a/t$  needs to be regulated to be within a certain range for a PTC thermistor in the present embodiment to obtain a sufficiently high rising rate in the resistance is described; where “ $a$ ” represents a distance between the first, second, third inner electrodes **55a**, **55b**, **55c** and the side electrode **53a**, or **53b**, “ $t$ ” represents a thickness of the conductive polymer **51**.

Samples were manufactured in accordance with the manufacturing method of present embodiment in the following manner: thickness “ $t$ ” of the conductive polymer was fixed to be 0.15 mm; while the distance “ $a$ ” was varied from 0.15 mm to 1.2 mm, at an interval of 0.15 mm. The electrolytic copper foils were patterned accordingly.

In order to confirm difference in the rising rate of the resistance caused by the varied distance “ $a$ ”, the samples were tested as follows.

Five samples each, with which the distance “ $a$ ” varies from 0.15 mm to 1.2 mm at an interval of 0.15 mm, were mounted on a printed circuit board to be measured with respect to the resistance/temperature characteristic, in the same manner as in the first embodiment. It is confirmed that the rising rate of the resistance is high when the value  $a/t$  is 3 or greater, especially when it is 4 or greater. It is also confirmed that the rising rate of the resistance does not substantially change where the value  $a/t$  is 6 or greater, and the initial (25° C.) resistance becomes high.

Next, another type of chip PTC thermistor samples were manufactured by providing the conductive polymer sheet **61** on both surfaces of the sheet **64**, and the laminate was heated and pressed, so that the outer electrodes **52a**, **52b** locate within the conductive polymer **51**. Then, it underwent the same manufacturing procedure as the above third embodiment, to have the chip PTC thermistor samples manufactured. FIG. 17 shows a cross sectional view of the chip PTC thermistor. Thickness “ $t$ ” of the conductive polymer **51** was fixed at 0.15 mm, while the distance “ $a$ ” was

varied from 0.15 mm to 1.2 mm at an interval of 0.15 mm. Electrolytic copper foils were patterned accordingly. Five samples each were tested in the same manner to measure the resistance at 25° C. and 125° C., and the rising rate of the resistance was calculated. The results confirm that, like in the earlier samples, the rising rate of the resistance becomes high when the value  $a/t$  is 3 or greater, especially when it is 4 or greater. It is also confirmed that when the value  $a/t$  is 6 or greater, the rising rate of the resistance does not show a substantial change, and the initial (25° C.) resistance becomes high.

Next, with an aim to improve reliability in the connection between the first outer electrode **52a**, the second outer electrode **52b**, the second inner electrode **55b** and the first side electrode **53a**, as well as that between the first and the third inner electrodes **55a**, **55c** and the second side electrode **53b**, following chip PTC thermistor samples were prepared. Namely, as shown in FIGS. 18(a) and (b), a first sub electrode **56a** is provided on a same plane of the outer electrode **52a**, sub electrode **56a** being independent from the outer electrode **52a** and connected with the side electrode **53b**. Also a second sub electrode **56b** is provided on a same plane of the outer electrode **52b**, sub electrode **56b** being independent from the outer electrode **52b** and connected with the second side electrode **53b**. Furthermore, a first inner sub electrode **57a** is provided on a same plane of the inner electrode **55a**, inner sub electrode **57a** being independent from the inner electrode **55a** and connected with the side electrode **53a**. Still further, a second inner sub electrode **57b** is provided on a same plane of the inner electrode **55b**, inner sub electrode **57b** being independent from the inner electrode **55b** and connected with the side electrode **53b**. Still further, a third inner sub electrode **57c** is provided on a same plane of the inner electrode **55c**, inner sub electrode **57c** being independent from the inner electrode **55c** and connected with the side electrode **53a**.

The samples were manufactured in the following manner: thickness “ $t$ ” of the conductive polymer **51** was fixed to be 0.15 mm; each of the respective distances between the sub electrode **56a** and the outer electrode **52a**, between the sub electrode **56b** and the outer electrode **52b**, between the inner sub electrode **57a** and the inner electrode **55a**, between the inner sub electrode **57b** and the inner electrode **55b**, and between the inner sub electrode **57c** and the inner electrode **55c** to be longer than 0.3 mm; and the distance “ $a$ ” between the first, second, third inner electrodes **55a**, **55b**, **55c** and the side electrode **53a**, or **53b**, was varied from 0.45 mm to 1.2 mm, at an interval of 0.15 mm. The electrolytic copper foils were patterned accordingly. Five samples each were tested in the same manner to measure the resistance at 25° C. and 150° C., and the rising rate of the resistance was calculated. The results confirm that, like in the earlier samples, the rising rate of the resistance becomes high when the value  $a/t$  is 3 or greater, especially when it is 4 or greater. It is also confirmed that when the value  $a/t$  is 6 or greater, the rising rate of the resistance does not show a substantial change, and the initial (25° C.) resistance becomes high.

In the present embodiment, the side electrode **53a** and the side electrode **53b** have been provided respectively as a first electrode and a second electrode. However, the locations for the first electrode and the second electrode are not limited to the side faces of the conductive polymer **51**. Instead, the first electrode and the second electrode can be a first penetrating through electrode **58a** and a second penetrating through electrode **58b** as shown in FIG. 19.

Namely, referring FIG. 19, the conductive polymer **51**, the outer electrode **52a**, the outer electrode **52b**, the protective

coatings 54a, 54b, the inner electrode 55a, the inner electrode 55b and the inner electrode 55c have been structured the same as those in the present embodiment. The difference as compared with the above third embodiment (FIG. 14) is that there are a first penetrating through electrode 58a which is electrically connected with the outer electrodes 52a, 52b and a second penetrating through electrode 58b which is electrically connected with the inner electrodes directly opposing to the outer electrodes. The above-configured chip PTC thermistors also provide the same effects as those of above third embodiment.

The shapes, materials and the like for the outer electrode, side electrode, inner electrode can be the same as in the first embodiment.

In the foregoing descriptions, a high density polyethylene has been used as the material for the crystalline polymer. However, as readily understood from the functioning mechanism, the material in the present invention is not limited to the high density polyethylene. The present invention can be applied in all the PTC thermistors that comprise polyvinylidene fluoride, PBT resin, PET resin, polyamide resin, PPS resin or the like crystalline polymers.

#### Industrial Applicability

The PTC thermistors of the present invention employ a conductive polymer having the PTC property, and a ratio a/t is regulated within a range 3-6; where "a" represents a distance between a first electrode, or a second electrode, and the adjacent inner electrode, while "t" represents a distance between each of the inner electrodes, or between the first, or the second, outer electrode and the adjacent inner electrode. With the above-described structure in accordance with the present invention, resistance of a PTC thermistor can be suppressed at a low level, so it is usable for large current applications. In addition, it provides a sufficient rate of the resistance rise. Thus the PTC thermistors in accordance with the present invention can effectively work to prevent an overcurrent in large current circuits.

What is claimed is:

1. A chip polymer PTC thermistor comprising:  
a conductive polymer having PTC properties;  
a first outer electrode in contact with said conductive polymer;  
a second outer electrode sandwiching said conductive polymer with said first outer electrode;  
one or more inner electrode disposed in between and parallel to said first and second outer electrodes, said one or more inner electrode being sandwiched by said conductive polymer;  
a first electrode directly electrically coupled with said first outer electrode; and  
a second electrode disposed electrically independently from said first electrode;  
wherein, when defining an inner electrode placed at the most adjacent to said first outer electrode as "one", and defining a "n"th inner electrode counting from the "one" as a "n"th inner electrode, odd-numbered inner electrodes are directly coupled with said second electrode and even-numbered inner electrodes, with said first electrode, and  
when the total number of said inner electrodes is an odd number, said second outer electrode is electrically directly coupled with said first electrode, whereas when it is an even number, coupled with said second electrode; wherein,

defining a distance from said odd-numbered inner electrode to said first electrode, or from said even-numbered inner electrode to said second electrode as "a", and a distance between the adjacent inner electrodes among said inner electrodes, or a distance between the inner electrode adjacent to said first outer electrode, or said second outer electrode, and said first outer electrode, or said second outer electrode, as "t", a ratio a/t is within a range 3-6, and

wherein said ratio a/t is increased by maintaining "t" and increasing "a" in order to increase resistance of said thermistor.

2. The chip polymer PTC thermistor of claim 1, wherein said first electrode is a first side electrode provided on one of the side faces of said conductive polymer, while said second electrode is a second side electrode provided on the other side face of said conductive polymer.
3. The chip polymer PTC thermistor of claim 1, wherein said first electrode is a first through electrode provided penetrating in said conductive polymer at one end, while said second electrode is a second through electrode provided penetrating in said conductive polymer at the other end.
4. The chip polymer PTC thermistor of claim 1, wherein said first electrode is a first side electrode provided on one of the side faces of said conductive polymer, said first side electrode making direct electrical contact with said first outer electrode and said even-numbered inner electrode, while said second electrode is a second side electrode provided on the other side face of said conductive polymer, said second side electrode making direct electrical contact with said odd-numbered inner electrode; and

when the total number of said inner electrodes is an odd number, said second outer electrode makes direct electrical contact with said first side electrode, whereas when the total number of said inner electrodes is an even number, said second outer electrode makes direct electrical contact with said second side electrode.

5. The chip polymer PTC thermistor of claim 1, wherein said ratio a/t is within a range 4-6.

6. A chip polymer PTC thermistor comprising:  
a conductive polymer having PTC properties;  
a first outer electrode in contact with said conductive polymer;  
a second outer electrode sandwiching said conductive polymer with said first outer electrode;  
one or more inner electrode disposed in between and parallel to  
said first and second outer electrodes and sandwiched by  
said conductive polymer;  
a first outer sub electrode disposed on a same plane with  
said first outer electrode, said first outer sub electrode  
being separated from said first outer electrode with a  
certain specific distance while being in contact with  
said conductive polymer;  
a second outer sub electrode disposed on a same plane  
with said second outer electrode, said second outer sub  
electrode being separated from said second outer elec-  
trode with a certain specific distance while being in  
contact with said conductive polymer;  
inner sub electrodes provided for a same number of said  
inner electrodes, each of said sub electrodes being  
disposed on same planes with said respective inner

**15**

electrodes and separated from said inner electrode with a certain specific distance while in contact with said conductive polymer;

a first electrode directly electrically coupled with said first outer electrode;

a second electrode disposed electrically independently from said first electrode, and making direct electrical contact with said first outer sub electrode;

wherein, when defining an inner electrode placed at the most adjacent to said first outer electrode as "one", and defining a "n"th inner electrode counting from the "one" as a "n"th inner electrode,

odd-numbered inner electrodes and even-numbered inner sub electrodes are directly coupled with said second electrode, and even-numbered inner electrodes and odd-numbered inner sub electrodes are directly coupled with said first electrode, and

when the total number of said inner electrodes is an odd number, said second outer electrode is electrically directly coupled with said first electrode, and said second outer sub electrode is electrically directly coupled with said second electrode,

when it is an even number, said second outer electrode is electrically directly coupled with said second electrode, and said second outer sub electrode is electrically directly coupled with said first electrode; wherein,

defining a distance from said odd-numbered inner electrode to said first electrode, or from said even-numbered inner electrode to said second electrode as "a", whereas a distance between the adjacent inner electrodes among said inner electrodes, or a distance between the inner electrode disposed next to said first outer electrode, or said second outer electrode, and said first outer electrode, or said second outer electrode, as "t",

a ratio a/t is within a range 3-6, and

wherein said ratio a/t is increased by maintaining "t" and increasing "a" in order to increase resistance of said thermistor.

7. The chip polymer PTC thermistor of claim 6, wherein said first electrode is a first side electrode provided on one of the side faces of said conductive polymer, while said second electrode is a second side electrode provided on the other side face of said conductive polymer.

8. The chip polymer PTC thermistor of claim 6, wherein said first electrode is a first through electrode provided penetrating in said conductive polymer at one end, while said second electrode is a second through electrode provided penetrating in said conductive polymer at the other end.

**16**

9. The chip polymer PTC thermistor of claim 6, wherein said first electrode is a first side electrode provided on one of the side faces of said conductive polymer, said first side electrode making direct electrical contact with said first outer electrode, said even-numbered inner electrode and said odd-numbered inner sub electrode, while said second electrode is a second side electrode provided on the other side face of said conductive polymer, said second side electrode making direct electrical contact with said first outer sub electrode, said odd-numbered inner electrode and said even-numbered inner sub electrode; wherein

when the total number of said inner electrodes is an odd number, said second outer electrode makes direct electrical contact with said first side electrode, and said second outer sub electrode makes direct electrical contact with said second side electrode, when the total number of said inner electrodes is an even number, said second outer electrode makes direct electrical contact with said second side electrode, and said second outer sub electrode makes direct electrical contact with said first side electrode.

10. The chip polymer PTC thermistor of claim 6, wherein said ratio a/t is within a range 4-6.

11. A thermistor, comprising:

- a polymer having conductive filler;
- first and second side electrodes on different sides of said polymer;
- an upper electrode extending from said first side electrode towards and spaced away from said second side electrode;
- an inner electrode extending from said second side electrode towards and spaced away from said first side electrode;

wherein said inner electrode is spaced away from said first side electrode by a distance "a", said inner electrode is spaced away from said upper electrode by a distance "t", and

wherein a/t is in the range of 3-6.

12. A thermistor according to claim 11 further comprising a further inner electrode extending from said first side electrode towards said second side electrode.

13. A thermistor according to claim 11, wherein a portion of said upper electrode is directly over at least a portion of said inner electrode.

14. A thermistor according to claim 11, wherein said inner electrode is buried in said polymer.

\* \* \* \* \*